

## UNITED STATES PATENT OFFICE

2,115,317

## IMPROVEMENTS IN THE DYEING OF TEXTILES

Karl Ott, Pavolding, and Otto Storb, Leverkusen-I. G. Werk, Germany, assignors to General Aniline Works, Inc., New York, N. Y., a corporation of Delaware

No Drawing. Application August 9, 1935, Serial No. 35,530. In Germany August 25, 1934

9 Claims. (Cl. 8—5)

The present invention relates to a process for the dyeing of textiles.

On dyeing delicate tissues with certain vat dyestuffs, particularly such of the anthraquinone series, the mechanical properties, i. e. strength and resistance, of the textile fibers are often impaired, especially, if during the dyeing process they are repeatedly exposed to reduction and oxidation by the change between vat and air. Damages of the kind described are often met with when dyeing delicate tissues of artificial silk or cotton fabrics for a prolonged time on the reel vat or of yarns on Seller's machine.

We have now found that the said fabrics can be excellently protected against this injurious action of certain vat dyestuffs by carrying out the printing or dyeing process in the presence of antioxidantizing agents. As such agents preferably phenolic products being easily converted into quinones as, for instance, hydroquinone, have proved to be satisfactory. Instead of antioxidantizing agents also such compounds may be employed which, during dyeing or printing, are transformed into antioxidantizing agents. In this respect, for instance, quinones of the benzene and naphthalene series have proved to be suitable; their protecting effect probably being due to the fact, that they are reduced by means of the reacting agents employed in the preparation of the vat and then behave like antioxidantizing agents. Besides hydroquinone or benzene quinone also naphthalene quinone sulfonic acid, tannin and like substances have proved to be suitable. In most cases already a very small quantity of the said protecting agents which may be used also in mixture with each other will be sufficient in order to obtain the desired effect. The protecting agents may be separately added to the dye bath or they can be incorporated with the dyestuff already ready before its use.

The following examples illustrate the invention:

*Example 1*

45 A cotton fabric (Setaline) is dyed for three hours on the reel with 20% of 2'3'6'7'-diphthalic-n-ethyl carbazole (10% paste) (s. Schultz-Julius, 7. Edn. No. 1286), the bath at the beginning containing per liter

50 4 gs. of the 10% dyestuff paste  
20 ecm. soda lye (38 Bé.)  
5 gs. of hydrosulfite.

The dyeing is carried out at a temperature of 55° C. in the usual way and hydrosulfite and lye are

subsequently added in the required amounts. During the dyeing the fabric loses more than 50% of its strength.

On repeating this experiment by adding 0.2 g. of tannin per liter to the dye bath, fabrics are obtained which have lost only 3.8% of their strength.

The same good result is obtained on adding instead of tannin 2 gs. of 1,4-naphthoic quinone sulfonic acid per liter of the dye bath.

The paste of this or other like injurious dyestuffs may also contain the necessary amount of tannin and/or 1,4-naphthoic quinone sulfonic acid beforehand.

*Example 2*

If a Setaline fabric is dyed with 20% of a 10% paste of 2'3'6'7'-diphthalic-n-ethyl-carbazole (s. Schultz-Julius, 7. Edn. No. 1286) in the presence of 0.2 g. hydroquinone per liter for three hours on the reel as described in Example 1, its strength practically remains unaltered. In contradistinction to the loss of 56.8% without the addition of hydroquinone, the strength is diminished only for 0.3%.

Instead of hydroquinone also 2 gs. of phenanthrene quinone per liter may be used with the same good result; both agents may also have been incorporated with the dyestuff before.

*Example 3*

A cotton fabric is dyed on the reel for three hours at 25° C. with 20% of a 10% paste of 1,2'-dianthraquinonylamine (s. Schultz-Julius, 7. Edn. Vol. I, No. 1249).

The dye bath contains per liter 5 gs. of the 10% paste of 1,2'-dianthraquinonylamine, 8 gs. soda lye of 38° Bé. and 5 gs. of hydrosulfite. The tensile strength of the dyed material is reduced for about 35%.

On adding 0.1 g. of hydroquinone per liter to the dye bath or using a dyestuff paste containing the respective amount of hydroquinone and dyeing in the same way, fabrics are obtained which show an unaltered tensile strength.

*Example 4*

Mercerized cotton yarn is dyed on Seller's machine with a dye bath according to Example 1, containing 0.5 g. of tannin per liter. The strength of the yarn is unimpaired, whilst without the addition of tannin it is diminished for about 15-35%.

We claim:

1. The composition of matter containing as es-

15

10

5

15

10

20

15

25

30

35

30

35

40

35

45

40

45

55

- sentient ingredients a vat dyestuff liable to damage cellulosic textile fibers during dyeing and an aromatic hydroxy compound capable of exercising an antioxidantizing action during the dyeing process.
- 5 2. In the process of dyeing textile material with a vat dyestuff liable to damage cellulosic textile fibers during dyeing the step which comprises dyeing in the presence of an aromatic hydroxy compound capable of exercising an antioxidantizing action during the dyeing process.
- 10 3. The composition of matter containing as essential ingredients a vat dyestuff liable to damage cellulosic textile fibers during dyeing and 15 hydroquinone.
4. The composition of matter containing as essential ingredients a vat dyestuff liable to damage cellulosic textile fibers during dyeing and a quinone.
- 15 20 5. The composition of matter containing as essential ingredients a vat dyestuff liable to damage
- cellulosic textile fibers during dyeing and naphthalene quinone sulfonic acid.
6. The composition of matter containing as essential ingredients a vat dyestuff liable to damage cellulosic textile fibers during dyeing and 5 tannin.
7. In the process of dyeing textile material with a vat dyestuff liable to damage cellulosic textile fibers during dyeing, the step which comprises dyeing in the presence of hydroquinone. 10
8. In the process of dyeing textile material with a vat dyestuff liable to damage cellulosic textile fibers during dyeing, the step which comprises dyeing in the presence of a quinone.
- 15 9. In the process of dyeing textile material with a vat dyestuff liable to damage cellulosic textile fibers during dyeing, the step which comprises dyeing in the presence of tannin.

KARL OTT. 20  
OTTO STÖRBE.